

## UNITED STATES PATENT OFFICE

2,217,422

## GLASS-METAL SEAL

Howard Scott, Forest Hills, Pa., assignor to Westinghouse Electric & Manufacturing Company, a corporation of Pennsylvania

No Drawing. Original application July 5, 1929, Serial No. 376,291, now Patent No. 2,062,335, dated December 1, 1936. Divided and this application April 24, 1936, Serial No. 76,199

4 Claims. (Cl. 49—92)

My invention relates to alloys and particularly to alloys of metals in the iron group of the periodic table.

This application is a division of my copending application Serial No. 376,291, filed July 5, 1929, which application issued on December 1, 1936, as Patent 2,062,335, and is assigned to the same assignee as this application.

One object of my invention is to provide an alloy having a predetermined coefficient of expansion over a temperature range from substantially room temperature to the annealing temperature of certain glasses, particularly ordinary lead glass.

Another object of my invention is to provide an alloy having a smaller coefficient of expansion than the nickel-steel alloys.

Another object of my invention is to provide an alloy adapted to form a vacuum-tight seal through lead glass.

Another object of my invention is to provide a method for producing a vacuum-tight seal of electrical conductors, having only a limited range of expansivity substantially equal to that of ordinary glasses, through the latter without causing breakage of the seals in cooling to room temperature.

Other objects of my invention will become apparent on reading the following specification.

In connection with the manufacture of vacuum-tight electrical-discharge devices in glass containers, the problem arises of making vacuum-tight seals of metals through the glass walls. In forming such seals, a small hole is melted in the glass wall of the container; the metal lead is inserted and the molten glass squeezed around the lead and fused thoroughly in contact therewith. In order that the resulting seal shall not crack or leak after it has cooled, it is necessary that the metal and the glass shall have substantially the same expansivity with temperature over the range from the annealing temperature of glass down to room temperature; and preferably that the metal be one which the glass will "wet." Platinum metal has the proper expansivity when used in combination with ordinary lead glass, and the first successful seals through glass were made with platinum leads.

Platinum is an extremely expensive metal and, consequently, composite conductors having cores of nickel-steel covered by thin jackets of copper were developed, and thus cheaper, but equally

satisfactory, seals through ordinary lead glass were obtained. The coefficient of expansion of copper is higher than that of lead glass; and, since the jacket of copper is relatively thin, the nickel-steel alloy employed is one which has a coefficient of expansion nearly equal to that of lead glass. Copper is a metal which lead glass "wets" readily; and the expansivity of nickel-steel is slightly less than that of glass over the range of approximately 400° C. between the temperature at which strains readily relieve themselves in lead glass and room temperature.

I find that, by employing certain other nickel-cobalt-iron alloys, and even certain nickel-iron alloys, seals may be made through ordinary lead glass; and this without the necessity for copper-jacketing the alloy.

In accordance with the foregoing principles, I have found that substitution of cobalt for nickel in nickel-iron alloys results in a decrease of expansivity of approximately  $0.5 \times 10^{-6}$  cm. per cm. per degree centigrade for each percent of cobalt thus substituted. Ordinary lead glass has an expansivity of approximately  $9 \times 10^{-6}$  cm. per cm. per degree C. while boro-silicate glasses have expansivities between 3.0 and  $7.0 \times 10^{-6}$  cm. per cm. per degree C.

In general, I have found that, in the case of alloys of low expansivity containing nickel and iron, whether or not they also contain cobalt, it is desirable that the relationship expressed by the following formula should hold.

$$\frac{\% \text{ nickel} + 2.5 (\% \text{ manganese}) + 18 (\% \text{ carbon})}{\% \text{ iron}} = 0.50 \text{ to } 0.60$$

the best value for the fraction being about 0.55. It also appears desirable, for most purposes, to minimize the amount of manganese, the maximum percentage of this element being preferably below 0.2%. Carbon, however, appears, in most instances, to be desirable up to the amount of 0.3%, as it permits a higher cobalt content than would otherwise be desirable and does not seriously affect expansivity.

As previously stated, I have found certain nickel-cobalt-iron alloys to seal successfully into ordinary lead glass having a coefficient of expansion in the neighborhood of  $9 \times 10^{-6}$  cm. per cm. per degree C. For instance, alloys comprising 30% to 45% nickel, 5% to 25% cobalt and 0 to 1% manganese, form satisfactory seals with lead glass having an expansivity between  $6 \times 10^{-6}$  and  $10 \times 10^{-6}$  cm. per cm. per degree C.

I have found that the preparation of vacuum-

tight seals between metals and glass is rendered more certain if the metals are annealed in vacuo or in a bath of a fused salt which readily dissolves the oxides of the metal. For example, 5 sodium nitrate is one such salt, many others being known to skilled chemists.

I have also found that a certain amount of trouble is caused in making vacuum-tight seals because of gases released at a high temperature, 10 and largely results from a reaction between carbon in the metal and oxide formed on the surface of the metal during heating in air.

This source of gas may be eliminated either by removing carbon from the metal or by coating 15 the metal with another metal which is impervious to oxygen and contains no carbon.

Small amounts of carbon cannot be avoided in iron-base alloys without elaborate precautions. Consequently, it is more convenient to remove 20 the carbon from the alloy than to prevent its introduction therein. Carbon may be removed from the molten alloy by maintaining it in a vacuum in contact with refractory oxides or by passing hydrogen through the metal. This treatment 25 is preferable when the finished piece is bulky. When, however, the metal is finished to a small cross-section, the carbon may be removed conveniently from the solid metal. The treatment required is heating at an appropriate temperature in hydrogen or in a fused salt bath containing no great amount of carbon compounds. A bath comprising 15% sodium chloride and 85% barium chloride at from 700° to 1200° 30 centigrade is one suitable bath.

35 Coating to avoid gas generation at the surface may be readily accomplished by electrolytic deposition of a thin layer of chromium or other carbon-free metal provided that the oxygen-carbon relations within the alloy are not such as to cause severe gas release at working temperatures. In the event that gas is evolved without 40 surface oxidation, a treatment, such as that just described, may first be applied to prevent injury to the coating by the gas. This treatment is particularly applicable to plated metals intended 45 for high-temperature service.

The temperature at which strains are readily relieved in glass is, of course, not an absolutely fixed quantity, even for glass of a given chemical 50 composition. At very high temperatures, the glass is relatively soft and, as the temperature decreases, it hardens. The lower the temperature and, consequently, the harder the glass, the less rapidly it is able to flex and relieve mechanical strains existing within it. However, since the in- 55

flection temperature, that is to say, the maximum temperature, at which coefficient of expansion of the above-described alloys remains low, decreases as the coefficient of expansion itself is decreased, it is desirable to form seals with as low an annealing temperature as possible. I have found that alloys, in which the inflection temperature is relatively low, may be employed to produce satisfactory seals if the completed seal is maintained at a temperature of about 50° C. above the 10 inflection temperature for a considerable period of time. Thus, while the strains are relieved slowly, they do so progressively and with certainty, and a strong vacuum-tight seal results in the end. 15

As an example of the softer glasses, referred to above as lead glasses, the following may be taken as typical in composition:

63.1%  $\text{SiO}_2$ ; 20.2%  $\text{PbO}$ ; 0.28%  $\text{Al}_2\text{O}_3$ ; 0.94%  $\text{CaO}$ ; 7.6%  $\text{NaO}$ ; 5.5%  $\text{K}_2\text{O}$ ; 0.88%  $\text{Mn}_3\text{O}_4$ . 20

The above subject-matter is also described and referred to in my copending application Serial No. 376,292, filed July 5, 1929, for Alloys, now Patent 1,942,260, issued January 2, 1934.

While I have, in the foregoing, described certain particular embodiments of my invention, it will be understood that these are for purposes of illustration only, and that the broad principles may be otherwise utilized, as will be readily apparent to those skilled in the art. 25

I claim as my invention:

1. A vacuum-tight seal between an alloy consisting of iron, nickel, cobalt and manganese and a glass containing substantially 63.1%  $\text{SiO}_2$ ; 20.2%  $\text{PbO}$ ; 0.28%  $\text{Al}_2\text{O}_3$ ; 0.94%  $\text{CaO}$ ; 7.6%  $\text{NaO}$ ; 5.5%  $\text{K}_2\text{O}$  and 0.88%  $\text{Mn}_3\text{O}_4$ . 30

2. A vacuum-tight seal between a glass containing substantially 63.1%  $\text{SiO}_2$ ; 20.2%  $\text{PbO}$ ; 0.28%  $\text{Al}_2\text{O}_3$ ; 0.94%  $\text{CaO}$ ; 7.6%  $\text{NaO}$ ; 5.5%  $\text{K}_2\text{O}$  and 0.88%  $\text{Mn}_3\text{O}_4$  and an alloy comprising 30 to 40 45% nickel, 5 to 25% cobalt, from a trace to 1% manganese and the remainder iron.

3. A vacuum-tight seal between a vitreous material having an expansivity of  $6.5 \times 10^{-6}$  cm. per cm. per °C., and an alloy comprising 43 to 45% nickel, 10 to 15% cobalt, from a trace to less than 1% manganese and the remainder iron. 45

4. A vacuum-tight seal between a vitreous material containing substantially 63.1%  $\text{SiO}_2$ ; 20.2%  $\text{PbO}$ ; 0.28%  $\text{Al}_2\text{O}_3$ ; 0.94%  $\text{CaO}$ ; 7.6%  $\text{NaO}$ ; 5.5%  $\text{K}_2\text{O}$  and 0.88%  $\text{Mn}_3\text{O}_4$  and an alloy comprising 43 to 45% nickel, 10 to 15% cobalt, from a trace to less than 1% manganese and the remainder iron. 50

HOWARD SCOTT. 55